

May 30, 1933.

E. GATHMANN

1,911,228

METHOD OF PRODUCING INGOTS

Filed July 6, 1932



## UNITED STATES PATENT OFFICE

EMIL GATHMANN, OF BALTIMORE, MARYLAND

## METHOD OF PRODUCING INGOTS

Application filed July 6, 1932. Serial No. 621,100.

This invention relates to methods of producing big-end-up ingots, and more particularly to methods of producing big-end-up ingots from fully-degasified or deoxidized steel, that is, ingots known to the art as "killed steel ingots". Apparatus suitable for use in carrying out my improved method is shown in my prior Patent No. 1,897,696, issued February 14, 1933, and in my copending application Serial No. 619,807 filed June 28, 1932.

Prior to the present invention, the greater tonnage of "killed steel ingots" has been produced in big-end-up castiron molds adapted to retard the solidification of the upper portion of the ingot relative to that of the lower portion and fitted with fireclay shrinkhead casings so as to confine the pipe or cavity incident to the shrinkage of the ingot metal from the liquid to the solid state to the extreme upper portion of the ingot. The shrinkhead portion of the ingot also provided a projection above the mold proper, making it possible to lift or strip the ingot with the soaking pit tongs, whereas without such a projecting portion the molds must be suspended and the ingots dumped.

The primary function of a shrinkhead casing is to retard the solidification of the upper portion of an ingot until the lower and intermediate portions have cooled and solidified thru the absorption of the heat of the forming ingot by the mold walls. While heretofore no satisfactory substitute had been found, the use of firebrick shrinkhead casings has a number of disadvantages. Being made of brick or loam, small particles of the shrinkhead casing at times break off and drop into the mold when the casing is being positioned on the mold, and it sometimes happens that the pouring ladle is not centered accurately over the mold and the stream of molten metal washes away a portion of the casing during teeming. In this way particles of the brick or loam are carried into the ultimate product. Furthermore, shrinkhead casings are expensive and increase materially the cost of sound ingot production.

Frequently, in order to reduce the depth

of pipe in the ingot, small quantities of heat-producing materials, such as straw, and occasionally heat-insulating substances, such as infusorial earth, have been thrown on the upper surface of the ingot to some advantage, but the value of complete insulation of the top surface of an ingot has not heretofore been fully realized. The practice of placing such material on the top surface of an ingot is disclosed for example in my Patent No. 1,711,052 of April 30, 1929.

In accordance with my present method, the use of shrinkhead casings in the production of most grades of steel is not essential or even desirable.

It will be understood that, when an ingot has been teemed, the walls of the forming mold expand due to the heat of the molten ingot metal within, and the solidifying ingot decreases in cross section due to the contraction incident to cooling. This results in the formation of an annular air space between the mold matrix and the sides of the ingot, this space being described in my Patent No. 983,357 of February 7, 1911. The air in this space is rarified and stagnant and serves to insulate the ingot from the mold and to retard the solidification of the ingot. This insulation is so effective that the one-fourth of the ingot volume last to solidify takes approximately as much time as the first three-fourths.

An object of the present invention is to provide a method for producing metallic ingots in such manner that the total time required for complete solidification of the ingot is materially reduced. In accordance with this method, the ingot is pushed up or partially stripped from the mold after a predetermined portion of the molten ingot mass has solidified and air is caused to flow thru the space between the ingot and mold matrix. It is important that the partial stripping of the ingot be performed at a time within a predetermined stage of solidification. Best results are obtained when the ingot is raised when between sixty and ninety percent of its volume has solidified, the time required for solidification varying with the square of the cross section of the mold cham-

ber. Heretofore ingots have been partially stripped from their molds before complete solidification of the metal, for example as shown in my Patent No. 1,059,668 of April 5 22, 1913, but in accordance with such prior practice, the ingot was stripped without particular reference to the degree of solidification and without providing for the rapid cooling of the ingot thru free circulation of 10 air between the mold and ingot. The primary purpose of early stripping as practiced in the prior art was to lower the cost of reheating the ingots by placing them in the soaking pits before complete solidification 15 and to lengthen the life of the molds.

Other objects will become apparent from a reading of the following description, the appended claims and the accompanying drawing, in which:

20 Figure 1 is a transverse vertical sectional view of apparatus for practicing my improved method, the illustrative embodiment comprising a mold support or car and an ingot mold supported thereon, the ingot 25 metal within the mold being shown graphically as in the initial stage of solidification;

Figure 2 is a view similar to Figure 1 but omitting the car and showing the ingot metal at a subsequent stage of solidification;

30 Figure 3 is a view similar to Figure 2 but showing the ingot partially stripped from the mold and in a late stage of solidification;

Figure 4 is a view similar to Figure 3 but showing the ingot as having solidified completely;

Figure 5 is a horizontal sectional view of a device for insulating the top surface of the ingot;

40 Figure 6 is a sectional view taken on the line 6—6 of Figure 5; and

Figure 7 is a graphic chart illustrating the comparative time phase of solidification of an ingot cooled entirely within the mold matrix and the time phase of solidification

45 of an ingot of the same cross section and volume produced in accordance with my present invention.

50 Referring to the apparatus shown by way of illustration as being suitable for use in practicing the method in accordance with the invention, a mold M of the big-end-up Gathmann type now well known to the art and shown for example in my Patent No. 1,806, 753 of May 26, 1931, is supported on a stool 55 S, which in turn is carried by a car C. The mold is provided with a necked-in tapered bottom opening 1, which is closed by means of spaced closure plugs 2 and 3. The stool is provided with an opening 4 in alignment with the opening 1 in the bottom of the mold, and the car is provided with an opening 5 in alignment with the openings 1 and 4.

60 A stripper rod 6 is mounted for sliding movements within the opening 5 in the car, and is adapted to be moved upwardly

through the openings 5, 4 and 1 into engagement with the closure plugs for moving the ingot relatively upward thru the mold. The stripper rod is provided with a longitudinally-extending groove 7, which receives for 70 sliding movements the inner end of a latch-rod 8, the latter being urged inwardly into engagement with the root of the groove 7 by a spring 9. The stripper rod is formed with notches 10 near the bottom of the groove 7, which are adapted to receive the inner end of the latch rod 8 when the stripper rod 6 has been raised and the ingot partially lifted or stripped from the mold to the desired extent.

75 The openings 1 in the mold and 4 in the stool preferably are considerably larger than the head of the stripper rod so as to provide for the passage of air up into the mold when the stripper rod and ingot are raised. In order to provide for the entrance of air into the openings referred to, the car is formed with a plurality of openings 11 directly under the stool. Apparatus of the 80 nature referred to above is described more in detail in my copending application Serial No. 619,807, filed June 28, 1932, and my Patent No. 1,897,696, issued February 14, 1933.

85 Referring now to the method employed in producing killed steel ingots in accordance with the invention, the well-deoxidized steel is poured in the usual manner into the mold M, which may or may not be fitted with a shrinkhead casing. Immediately after teeming the ingot to the required level below the top of the mold, a measured quantity of refractory heat-insulating material 12 is placed on the surface of the molten metal. This material preferably comprises thoroughly dried, 90 finely-divided diatomite or infusorial earth.

95 Shortly after the metal has been poured, the chilling effect of the iron will cause the ingot metal which is in contact with the bottom and walls of the mold to solidify, the initial stage of solidification being shown in Figure 1, wherein the chilled solidified portion of the ingot metal is indicated at 13, the molten metal is indicated at 14, and the heat-insulating material on top of the ingot metal is indicated at 12.

100 The ingot metal is allowed to solidify further until approximately sixty to ninety percent of the metal has solidified, at which time the formation of the partially solidified ingot and the remaining molten metal will be substantially as shown in Figure 2. It will be noted that when the solidification reaches this stage, a small annular air chamber will have been formed between the ingot metal and the mold due to the expansion of the mold and the contraction of the ingot.

105 In accordance with the prior practice generally followed, the ingot is left in the mold until completely solidified. Due to the in-

sulation afforded by the air space, solidification is very slow after the formation of this space and it is necessary to leave the ingots in the molds for a relatively long time to insure complete solidification. As much as two hours is required for the solidification of an ingot of 22" cross section by this method. This means that the molds are tied up, production is delayed and axial segregation of the metalloids—carbon, sulphur, phosphorous and the like—is increased in the slowly cooling ingot.

In accordance with the present invention, when the solidification has taken place throughout a predetermined volume of the ingot metal, between sixty and ninety percent and preferably about 75% thereof, the stripper rod 6 is raised by any suitable means, such for example as those shown in the co-pending applications referred to, in order to raise or strip the ingot partially from the mold. The position of the ingot after this partial stripping operation is shown in Figure 3 and it will be noted that the upper portion only of the ingot has been moved up beyond the top of the mold. When the ingot is in this position, relatively cool air is caused to flow upwardly thru the openings 11 in the car, the openings 4 in the stool and the opening 1 in the mold and into the bottom of the mold chamber. The air, becoming highly heated and rarified by contact with the hot mold walls and the hot ingot, automatically flows upwardly through the annular gap between the ingot and mold very rapidly, due to the draft created by the heating of the air. It is apparent that the entering air contacting with the bottom portions of the ingot will be relatively cooler as compared to the air which has been in contact with the bottom of the ingot and which has passed along the ingot, the result being that the air contacting with the ingot has a cooling effect on the latter which is progressively less from the bottom to the top of the ingot. This results in more rapid heat abstraction and consequent quicker solidification of the lower and intermediate portions of the ingot than of its upper portions, so that the formation of a deep-seated shrinkage cavity or pipe within the body of the ingot is prevented. In other words, the ingot metal is caused to cool and solidify more rapidly and yet progressively from the bottom towards the top. It is to be understood that progressive solidification from bottom to top is absolutely necessary to insure physical soundness in the ingot product. When the solidification of the ingot is complete, the vertical cross section of the ingot will be substantially as graphically shown in Figure 4, wherein it will be noted that the shrinkage cavity is confined to the extreme upper part of the ingot.

65 The time phase of solidification of ingots

made in accordance with the prior art and with my present method is illustrated graphically in Figure 7. The vertical lines  $T$ ,  $T^1$ ,  $T^2$ ,  $T^3$  and  $T^4$  designate successive intervals of time during solidification and the horizontal lines  $V$ ,  $V^1$ ,  $V^2$ ,  $V^3$  and  $V^4$  designate the volumes of metal solidified. The solid inclined line  $K$  shows the relative rate of solidification of an ingot when inclosed by the mold during its entire period of solidification. It will be noted that approximately 75% of the ingot has solidified at  $T^1$  where the air chamber is completely formed, when the rate of cooling is abruptly retarded, as shown by the inclination of the line  $K$  from its point of intersection with lines  $T^1$  and  $V^3$ . In my new method, the line  $K^1$  runs coincident with the line  $K$  for about 75% of its length, at which time the ingot is stripped or lifted up a predetermined distance and air is induced to flow thru the chamber between the mold and ingot. Cooling then proceeds at approximately the same rate as before the formation of the air gap, as indicated by the line  $K^1$ . The time of complete solidification of both types of ingots is indicated by the intersection of the cooling lines  $K$  and  $K^1$  with the time lines  $T^4$  and  $T^2$  respectively.

70 My new method is particularly advantageous when it is desired not to use shrinkhead casings, but may be used in connection with such casings if their use in the production of the particular type of steel being poured is considered desirable.

75 My new method is particularly advantageous when it is desired not to use shrinkhead casings, but may be used in connection with such casings if their use in the production of the particular type of steel being poured is considered desirable.

80 A properly designed big-end-up mold without a shrinkhead casing or other provision for insulation of the top of the ingot will produce an ingot having a relatively deep, funnel-like pipe or shrinkage cavity, necessitating a top crop of at least eighteen or twenty percent of the ingot volume, whereas, by practicing the method of the present invention, it is possible to reduce the depth of the shrinkage cavity to the top eight to twelve percent of the ingot volume. Not only is progressive solidification of an ingot thus accomplished without the use of a shrinkhead casing, but the total time required for the metal to solidify is reduced very materially, as graphically shown in Figure 7, thereby releasing the mold for further use and lengthening its life.

85 In order to obtain the full advantages of my process, it is desirable that the insulating material 12 placed on the top of the ingot metal be as moisture-free as practical and that a sufficient amount be used to at least completely fill the shrinkage cavity as it forms due to the contraction incident to solidification. In prior practice, whenever material to conserve the heat of the ingot has been placed on the top of the ingot, it has been usual for an unskilled laborer simply to throw an indeterminate and usually insufficient quantity of the material from a

130

shovel or the like. The material having been taken from a pile on the pouring floor or from an open container, contains a considerable amount of moisture, which varies 5 with the humidity of the air and which tends to chill the top of the forming ingot. Experience has demonstrated that for the best results the heat-insulating material should be as dry as possible and should have a depth 10 of from about one-quarter to three-quarters of the minimum cross section D of the ingot at its top, as shown in Figure 6 of the drawing. For instance, where the ingot has a cross sectional dimension of  $20 \times 22''$ , the 15 depth or thickness of the blanket of heat-insulating material should be at least 5" and usually need not exceed 15", the specific depth being dependent upon the temperature and analysis of the steel being poured. In 20 order that the material applied to the top of the ingot in practicing my method be as moisture-free as possible and in order to insure the use of a sufficient amount, I prefer to employ a substantially moisture-proof 25 carton—a paper bag or the like—filled with a measured quantity, two to six percent of the volume of the ingot metal, of dry, loose, finely-divided material, preferably diatomite or infusorial earth, which is readily obtainable, 30 inexpensive and when dry is one of the best non-conductors of heat known for the purpose. One embodiment of this device is illustrated in Figures 5 and 6, wherein a jacket 15 of moisture-proof, combustible material is 35 shown filled with a quantity of loose, finely-divided heat insulating material. For certain types of steel, this material may comprise an admixture of comminuted straw and diatomite or the like. When the ingot 40 metal has been poured, the carton containing the measured quantity of insulating material is at once deposited bodily on the top surface of the fluid ingot metal, whereupon the jacket 15 will be burned and the material 12 45 will be deposited substantially evenly over the surface of the molten metal, as shown in Figure 1 of the drawing. The upper contacting surface of the ingot will then remain molten and will feed the contracting ingot 50 to compensate for the shrinkage of the lower portions, until the entire mass has cooled and solidified progressively from bottom to top. When solidification is complete, the shrinkage cavity should be substantially full of the 55 heat-insulating material. If desired, this heat-insulating material may be retrieved and used again in accordance with the method shown and described in my Patent No. 1,719,542 of July 2, 1929. The top of the 60 ingot, being considerably extended above the top of the mold, is readily engageable by the soaking pit tongs or other apparatus for removing the ingot from the mold.

Although I prefer to employ means such 65 as are illustrated herein for facilitating the

depositing of the desired predetermined quantity of dry heat insulating material on top of the ingot metal, it is obvious that my improved method may be practiced without using the specific means described above. 70 The insulating means is disclosed and claimed in a division of the present application, filed September 26, 1932, Serial No. 634,950.

Due to the complete insulation of the top 75 of the ingot and the rapid cooling effected by the air draft during the later stages of solidification by this new method, it is possible to obtain a sounder and more homogeneous ingot structure than has been possible in prior 80 practice. The rapid cooling of the ingot decreases segregation to the minimum and lengthens the life of the mold, allowing of the production of a greater number of ingots 85 in the mold. By this new method, the danger of non-metallic inclusions in the ingot resulting from chipping or spawling of shrinkhead casings is eliminated and a superior product is produced at comparatively 90 low cost.

I claim:

1. The method of producing big-end-up metallic ingots which consists in pouring molten metal into a big-end-up mold, then 95 raising the ingot only partially through the mold as soon as the ingot-forming metal has solidified through sixty to ninety per cent of its volume, admitting air from the outside of the mold to the bottom of the annular space 100 between the mold and ingot, and supporting the ingot in said partially raised position until solidification is complete.

2. The method of producing big-end-up metallic ingots which consists in pouring molten metal into a big-end-up mold, covering 105 the top surface of the molten metal with heat-insulating material, then raising the ingot only partially through the mold as soon as the ingot-forming metal has solidified throughout sixty to ninety per cent of its volume, admitting air from the outside of the mold to the bottom of the annular space between the mold and ingot, and supporting the ingot in said partially raised position until 110 solidification is complete.

3. The method of producing big-end-up ingots from well deoxidized steel which consists in pouring the steel into a big-end-up mold, then raising the ingot only partially 115 through the mold as soon as the ingot-forming metal has solidified throughout substantially seventy-five per cent of its mass, admitting air from the outside of the mold to the bottom of the annular space between the mold and ingot, and supporting the ingot in said partially raised position until solidification is complete.

4. The method of producing big-end-up metallic ingots which consists in pouring molten metal into a big-end-up mold, then 120

raising the ingot only partially through the mold until the top portion of the ingot projects above the mold and with the bottom portion of the ingot still extending down into the mold as soon as the ingot-forming metal has solidified throughout sixty to ninety per cent of its volume, admitting air from the outside of the mold to the bottom of the annular space between the mold and ingot, and supporting the ingot in said partially raised position whereby cool air will flow into the bottom of the mold and up through the annular space between the mold and ingot for cooling the latter at a progressively decreasing rate from the bottom to the top thereof.

In testimony whereof, I have hereunto subscribed my name.

EMIL GATHMANN.

20

25

30

35

40

45

50

55

60

65